

## UNITED STATES PATENT OFFICE

2,052,873

PROCESS OF CARROTTING FUR AND THE  
LIKE AND COMPOSITION THEREFOR

Constantine F. Fabian, Brookfield, Conn., and  
Alexander N. Sachanen, Luxemburg, Luxemburg, assignors, by mesne assignments, to The  
Non-Mercuric Carrot Company, Danbury, Conn., a corporation of Connecticut

No Drawing. Application February 13, 1935,  
Serial No. 6,388

3 Claims. (Cl. 8—21)

This invention relates to the treatment of fur and similar animal fibers (herein generically designated as fur), and more especially to give such fur improved felting properties, and said invention further relates to a composition of matter adapted to be employed in such treatment.

In its natural state animal fur has inadequate felting properties and, as is well-known, preliminary to the formation of a suitable fur felt to be used in the manufacture of such articles as hats, must be subjected to a chemical treatment ordinarily termed "carrotting" to impart thereto the requisite felting properties. The procedure commonly adopted is to brush the carrotting solution into the fur while the latter is still on the skin, the latter being then set to one side to allow the fur to dry and the fur being thereafter removed from the skin and made into felt.

The object of the present invention, among other things, is to so improve the carrotting treatment and the carrotting solution employed in such treatment that, while the fur has imparted to it the property of rapid felting and the capacity of producing a tight, strong felt, certain objectionable features which have been inherent in processes heretofore in use are eliminated in whole or in part as will be better understood from the following.

The carrotting process is dependent on the action of chemical reagents which so act chemically on the surface of the animal fibers that the latter acquire felting properties previously absent, and, when subjected to hot water and pressure, tend to work into a closely interlocked relation with the resultant formation of a compact, tight, firm body of felt.

The process of carrotting comprehends not only a cleansing of the animal fibers from fats and other substances, the presence of which interferes with felting, but also chemical reactions of the carrotting reagents on the proteids of the fibers. This reaction is understood to proceed from a hydrolyzing and an oxidizing action.

Thus, it is well known that strong acids, such as sulphuric acid, impart some carrotting effect to animal fibers, but it is also known that sulphuric acid and other strong acids which are non-oxidizing produce only a hydrolyzing action. It is therefore apparent that a hydrolyzing action of acids on the fur is one of the chemical reactions which takes place in carrotting. But the carrotting effect alone of the strong acids of the class indicated is very weak and insufficient. The carrotting action is much more effective in the presence of an oxidizing agent and especially in

combination with a catalyst. Accordingly, an oxidizing action appears to be a chemical action in carrotting, these two reactions,—hydrolyzing and an oxidizing action,—on the fur fibers producing the so-called carrotting effect.

The carrotting treatment heretofore most commonly employed has been through the application to the fur of a carrotting solution containing a mixture of nitric acid and mercuric nitrate. In this case the nitric acid acts simultaneously as an acid and as an oxidizing agent, producing a hydrolyzing and oxidizing reaction on the animal fibers, while the mercuric nitrate has a catalytic action on the oxidizing process. At certain concentrations of these two reagents felting properties can usually be imparted to the fur.

This method of carrotting, however, has certain material defects and objections, among which are the following.

Unless carried out under carefully regulated conditions, difficult or impossible at all times to meet, the process tends to weaken the strength of the animal fibers, and furthermore to so change their structure that they lose in part their ability of fixing dye stuffs, with the result that such treated fibers tend to give off the dyes when washed.

In this process the hydrolyzing and oxidizing actions are effected by the same reagent,—nitric acid,—the oxidizing action of which takes place only at high concentrations. Under high concentrations its hydrolyzing action becomes so effective that it is apt to attack or partially destroy the animal fibers. Accordingly, great care has to be exercised in controlling the strength of the solution so that, on the one hand, it will be of sufficient strength to give the fur adequate felting properties while, on the other hand, it will not be so strong as to impair the quality of the fur.

This difficulty is increased by the fact that, after the solution has been brushed on the fur and the skins are set aside for drying, and as the drying proceeds, the nitric acid becomes stronger and more concentrated and acquires an increasing and greatly intensified oxidizing effect. Such intensified oxidizing effect tends to detrimentally affect the fibers unless carried out under carefully regulated physical drying conditions, within definitely maintained limits of temperature, humidity, etc., which conditions it is difficult or impracticable to strictly regulate.

Another objection is that the preparation of the commonly used carrotting solution, in which metallic mercury is dissolved in nitric acid, is a relatively slow process, taking a substantially long

time, and such preparation involves the emission of heavy brown vapors of lower oxygen compounds of nitrogen which are noxious and dangerous to health. The drying of the skins after the application of the solution of mercury nitrate in nitric acid also involves the emission of noxious vapors of nitric acid.

A further objection lies in the fact that on treating white or light colored animal fibers by the mixture of nitric acid and mercuric nitrate, the fibers change color and become yellow or red. This discoloration can be explained by the specific action of nitric acid and of mercuric nitrate on proteids; the latter turn yellow on heating with nitric acid and become red on heating with a solution of mercuric nitrate and nitric acid (Millon's test).

The use of two oxidizing agents in a carroting solution, as, for example, nitric acid and hydrogen peroxide, tends to eliminate the discoloration of white or light colored animal fibers. In such case the hydrogen peroxide oxidizes and destroys the pigments on the fibers formed by the action of nitric acid and mercuric nitrate. The use, however, of two energetic agents, such as nitric acid and hydrogen peroxide, in the same carroting solution tends to produce inordinately strong oxidation of the animal fibers which is difficult to control, with the result that the strength of the fibers as well as their affinity for dye stuffs tends to be detrimentally affected. Moreover, the use of hydrogen peroxide and nitric acid often produces yellow colored fibers on the edges of the skins, the intensity of which discoloration depends upon the drying conditions, such as temperature, humidity, etc., which are again difficult or impracticable to control. Furthermore, a carroting solution containing nitric acid and hydrogen peroxide cannot be stored and kept without losing much of its strength and effectiveness and must therefore be applied to the fur soon after its preparation.

Other carroting compositions have been suggested involving the use of oxidizing agents in an alkaline medium, as, for example, hydrogen peroxide in a sodium hydroxide solution. Treatments by such alkaline mediums, however, have been found to act destructively and detrimentally on the fibers of the fur.

Other methods of carroting have been suggested involving the use of sulphuric acid alone or a mixture of sulphuric acid with an oxidizing agent. These methods avoid discoloration of white animal fibers but are not sufficiently effective to produce an adequate carroting effect on the fibers unless concentration of the reagents is very high, and high concentration of such reagents as sulphuric acid or hydrogen peroxide acts detrimentally on and affects the strength of the treated fibers. The use of high concentrated sulphuric acid solutions especially tends to destroy the animal fibers in the course of the drying process as the sulphuric acid reaches stages of more intense concentration.

Through our improved carroting treatment, fur may be adequately and satisfactorily carroted, avoiding in whole or in part numerous objections and defects in prior carroting processes.

We have found that fur can be easily and satisfactorily carroted without the use of nitric acid or mercuric nitrate but through the use of a solution containing a non-oxidizing mercury salt (in which anion  $\text{NO}_3^-$  is absent) to serve as the catalyzing agent together with a hydrolyzing and non-

oxidizing acid and a suitable substantially non-hydrolyzing oxidizing agent.

In this carroting treatment, neither the mercury salt nor the acid has any sensible oxidizing effect so that the oxidizing and the hydrolyzing actions are separated and effected by different reagents. Accordingly, both the oxidizing and the hydrolyzing action of the carroting solution can be precisely regulated by the concentration of the oxidizing agent, the concentration of the mercury salt as a catalyst on the oxidization and the concentration of the acid as a hydrolyzing agent.

The catalytic action of mercury in carroting fur appears to be superior to that of other known catalysts and to have the property of giving to the felt a high quality of smoothness and softness of feel. We have found, however, that similar catalytic properties are provided by soluble mercury salts other than those containing the anion  $\text{NO}_3^-$ .

We have found that the required catalytic effect is obtained not only from such salts as mercuric sulphate, mercuric chloride, etc., which give the same ions as mercuric nitrate, but also from complex mercury salts, such as mercuric ammonium chloride or double salt of mercuric chloride and potassium chloride ( $\text{K}_2\text{HgCl}_4$ ), or similar salts, which give complex ions  $\text{HgNH}_2^-$  or  $\text{HgCl}_4^-$ , etc.

The employment of certain complex mercury salts as catalysts in carroting compositions is desirable since such salts as a rule are less harmful as contrasted with salts which give a two valent ion of mercury and may be used in preparation of the solution and in its application to the fur without much of the danger to health which has accompanied the use of mercuric nitrate.

As examples of non-oxidizing mercury salts, accordingly, we may use in practice such salts as mercuric sulphate, mercuric chloride, mercuric ammonium chloride, double salt of mercuric chloride and potassium chloride. The composition need not be confined to a single salt but mixtures of two or more mercury salts of the class indicated may be employed.

As acids we may use in practice any one or more of a group of stable acids capable of providing a non-oxidizing, hydrolyzing action. Among the inorganic acids which may be used for this purpose are sulphuric, hydrochloric, phosphoric and metaphosphoric acids which, under normal conditions, do not have an oxidizing effect. Hydrochloric acid not containing any oxygen has no oxidizing action. Sulphuric acid and phosphoric acid are formed of high oxygen compounds of sulphur and phosphorus which are among the most stable of the different compounds of these elements. For this reason these acids do not give any oxidization. Nitric acid, on the contrary, is formed of a very unstable, high compound of oxygen which readily decomposes into lower oxygen compounds with the liberation of oxygen and with corresponding oxidizing effect.

Instead of the more expensive phosphoric acid (pure acid 85%), the mixture of sulphuric acid or hydrochloric acid with binatriumphosphate (or other soluble salt of the same acid) can be used as this mixture gives relatively inexpensive phosphoric acid according to the following equation:



Or the solution of phosphoric acid can be ob-

tained by the reaction between calcium phosphate and sulphuric acid according to the following equation:



Calcium sulphate formed in this reaction can be easily removed by filtration.

- Sulphuric acid has a stronger hydrolyzing action than hydrochloric acid which is evidently the result of its non-volatility and therefore has a more prolonged and increasingly pronounced action upon the animal fibers during the drying stage. Accordingly we employ sulphuric acid in lower concentrations than hydrochloric acids. On the other hand, non-volatile but relatively weak phosphoric acid can be used in greater concentrations in carressing solutions.

The use of different acids permits treatment of the fur at different values of pH and at different volatile properties of the acids employed. The most favorable chemical conditions may be chosen, depending on the individual properties of the animal fibers to be treated. Mixtures of the various acids may also be employed to advantage. For example, a mixture of volatile hydrochloric acid and non-volatile sulphuric or phosphoric acid may be employed to good effect. The hydrolyzing effect of such a mixture is strong in the initial steps of carressing when and immediately after the solution is applied to the fur but diminishes rapidly at the drying stage due to the evaporation of the hydrochloric acid. The amount of sulphuric acid (or phosphoric acid) in such a mixture remaining on the fibers may be so chosen as to be insufficient to act detrimentally on the fibers and, on the contrary, to act favorably during the subsequent felting operation. Such a mixture avoids the possible ill effects of the sulphuric acid alone in cases where the carressed skins are to be held in storage for a substantial period of time before being put to use.

Besides inorganic acids, use may be made of organic acids which are soluble in water and are capable of producing non-oxidizing, hydrolyzing effects. Among such organic acids in common use and relatively inexpensive are formic, oxalic, and various chloroacetic and sulphonic acids. In the use of such organic acids it is sometimes advisable to mix the organic acid with one or more of the inorganic acids of the class previously mentioned in order to facilitate the solubility of the mercury salts.

As oxidizing agents we may employ such substantially non-hydrolyzing substances as chlorates, persulphates, inorganic and organic peroxides, etc.

The application of the carressing solution to the animal fibers may be carried out in the usual manner, which comprises brushing the solution into the fur while the latter is still on the skin. It may, however, be applied to the fur by spraying it on the fur while still on the skin or the fur itself, after having been cut from the skin, may have the carressing solution applied by immersion or otherwise. In the latter case the concentrations of the reagents should be materially reduced as compared to the concentrations used when the solution is applied by brushing or spraying on the fur while still on the skin.

The invention will be better understood by the following specific illustrated examples of various carressing solutions which may be prepared according to the principles of our invention and intended each for application to the animal fibers while still on the skins.

In each of the following examples the carressing composition comprises an aqueous solution having 100 parts by weight of water together with the chemical reagents named, in the proportions named, which proportions are also given in parts by weight.

#### Example 1

|                    | Parts |
|--------------------|-------|
| Mercuric chloride  | 3     |
| Sulphuric acid     | 3 10  |
| Potassium chlorate | 5     |

#### Example 2

|                   | Parts |
|-------------------|-------|
| Mercuric sulphate | 3     |
| Hydrochloric acid | 9 15  |
| Natrium peroxide  | 4     |

#### Example 3

|                            | Parts |
|----------------------------|-------|
| Mercuric ammonium chloride | 4 20  |
| Hydrochloric acid          | 4     |
| Sodium persulphate         | 5     |

#### Example 4

|                                              | Parts |
|----------------------------------------------|-------|
| Double salt K <sub>2</sub> HgCl <sub>4</sub> | 4 25  |
| Hydrochloric acid                            | 5     |
| Acetylperoxide                               | 5     |

#### Example 5

|                            | Parts |
|----------------------------|-------|
| Mercuric ammonium chloride | 5     |
| Phosphoric acid            | 8     |
| Sodium persulphate         | 6     |

#### Example 6

|                            | Parts |
|----------------------------|-------|
| Mercuric ammonium chloride | 5     |
| Sulphuric acid             | 8     |
| Sodium biphosphate         | 12    |
| Hydrogen peroxide          | 4 40  |

#### Example 7

|                            | Parts |
|----------------------------|-------|
| Mercuric ammonium chloride | 4     |
| Phosphoric acid            | 6     |
| Hydrochloric acid          | 2 45  |
| Potassium chlorate         | 6     |

#### Example 8

|                                              | Parts |
|----------------------------------------------|-------|
| Double salt K <sub>2</sub> HgCl <sub>4</sub> | 4     |
| Hydrochloric acid                            | 3 50  |
| Sulphuric acid                               | 1     |
| Hydrogen peroxide                            | 4     |

#### Example 9

|                            | Parts |
|----------------------------|-------|
| Mercuric ammonium chloride | 4     |
| Hydrochloric acid          | 3     |
| Formic acid                | 5     |
| Sodium persulphate         | 6     |

#### Example 10

|                                              | Parts |
|----------------------------------------------|-------|
| Double salt K <sub>2</sub> HgCl <sub>4</sub> | 4     |
| Hydrochloric acid                            | 3     |
| Oxalic acid                                  | 6     |
| Potassium chlorate                           | 8 65  |

In general, the proportions of mercury salts should comprise from one to eight parts by weight, those of the inorganic acids from one to twelve parts by weight, depending on their hydrolyzing strength, and those of the organic acids, which as a class have a lesser hydrolyzing strength, from one to twenty-five parts by weight.

The use of the described treatment not only provides a thoroughly carressed fur capable of pro-

ducing a fast-shrinking, tight and smooth felt, but also yields certain advantages, among which are the following:

The solution may be easily and quickly prepared. Its preparation and its application may be carried out without the production of noxious or poisonous vapors. In most of the examples previously given, the solution may be kept or stored for a substantial period of time without deterioration.

The described treatment effects no reduction in the affinity of the animal fibers for dye stuffs but insures a permanency in the dyes.

The described treatment does not discolor the fur fibers but leaves light colored or white carotted fur with its original, natural color unimpaired.

By proper selection of the strength of the acid reagent or reagents in solution, adequate and thorough carrotting is had without affecting the strength or otherwise impairing the desirable qualities of the animal fibers. Precautions required to control the carrotting effect in the case of the carrotting solution produced from nitric acid and mercuric nitrate are not required by the carrotting treatment by our process. The drying of the skins and the setting of the carrott may be effected without particular regard to temperatures and other drying conditions, and the skins may be stored for long periods of time without deterioration. Drying may be effected under the normal factory temperatures prevailing either in winter or summer, or may be effected at relatively high drying temperature. Drying of carotted animal fibers at high drying temperatures in the presence of strong non-volatile acids, such as sulphuric acid, tends to change the color and partly destroy the fibers. The use of our composition, when employing inorganic acids which are relatively volatile, such as hydrochloric acid, or relatively weaker acids, such as phosphoric acid, and also relatively weak stable organic acids, such as formic, acetic oxalic and chloroacetic acids, permits the fibers to be dried at high drying temperatures, thereby

shortening the time of drying and materially reducing the time required for the carrotting treatment in its entirety.

Various changes in and departures from the embodiments of our carrotting composition may be made as the same have been hereinbefore exemplified, all within the scope and principles of our generic invention, and it is understood that the matter hereinbefore set forth is submitted as illustrative and not in a limiting sense.

We claim:

1. The process of preparing fur or the like for felting, which consists in subjecting the fur to the action of an aqueous carrotting solution of a substantially non-hydrolyzing oxidizing agent, a non-oxidizing acid capable of a substantial hydrolyzing action on the fur, and one or more non-oxidizing mercuric salts soluble in water of the group consisting of mercuric chloride, mercuric sulphate, mercuric ammonium chloride and double salts of the type  $K_2HgCl_4$ .

2. As a composition of matter for the carrotting of fur or the like, an aqueous carrotting solution containing a substantially non-hydrolyzing oxidizing agent, a non-oxidizing acid capable of a substantial hydrolyzing action on the fur, and one or more non-oxidizing mercuric salts soluble in water of the group consisting of mercuric chloride, mercuric sulphate, mercuric ammonium chloride and double salts of the type  $K_2HgCl_4$ .

3. As a composition of matter for the carrotting of fur or the like, an aqueous solution containing an oxidizing agent, a non-oxidizing acid capable of a substantial hydrolyzing action on the fur, and one or more non-oxidizing mercuric salts soluble in water of the group consisting of mercuric chloride, mercuric sulphate, mercuric ammonium chloride and double salts of the type  $K_2HgCl_4$ , said solution having the proportions represented by 100 parts by weight of water, from 8 to 25 parts by weight of said acid, and from 1 to 8 parts by weight of mercuric salt.

CONSTANTINE F. FABIAN.

ALEXANDER N. SACHANEN.

45

#### CERTIFICATE OF CORRECTION.

Patent No. 2,052,873.

September 1, 193

CONSTANTINE F. FABIAN, ET AL.

It is hereby certified that error appears in the printed specification of the above numbered patent requiring correction as follows: Page 4, second column, line 33, claim 3, strike out "an" and insert instead the words a substantially non-hydrolyzing; and that the said Letters Patent should be read with this correction therein that the same may conform to the record of the case in the Patent Office.

Signed and sealed this 13th day of October, A. D. 1936.

Henry Van Arsdale  
Acting Commissioner of Patents.

(Seal)

ducing a fast-shrinking, tight and smooth felt, but also yields certain advantages, among which are the following:

The solution may be easily and quickly prepared. Its preparation and its application may be carried out without the production of noxious or poisonous vapors. In most of the examples previously given, the solution may be kept or stored for a substantial period of time without deterioration.

The described treatment effects no reduction in the affinity of the animal fibers for dye stuffs but insures a permanency in the dyes.

The described treatment does not discolor the fur fibers but leaves light colored or white carotted fur with its original, natural color unimpaired.

By proper selection of the strength of the acid reagent or reagents in solution, adequate and thorough carrotting is had without affecting the strength or otherwise impairing the desirable qualities of the animal fibers. Precautions required to control the carrotting effect in the case of the carrotting solution produced from nitric acid and mercuric nitrate are not required by the carrotting treatment by our process. The drying of the skins and the setting of the carrott may be effected without particular regard to temperatures and other drying conditions, and the skins may be stored for long periods of time without deterioration. Drying may be effected under the normal factory temperatures prevailing either in winter or summer, or may be effected at relatively high drying temperature. Drying of carrotted animal fibers at high drying temperatures in the presence of strong non-volatile acids, such as sulphuric acid, tends to change the color and partly destroy the fibers. The use of our composition, when employing inorganic acids which are relatively volatile, such as hydrochloric acid, or relatively weaker acids, such as phosphoric acid, and also relatively weak stable organic acids, such as formic, acetic oxalic and chloroacetic acids, permits the fibers to be dried at high drying temperatures, thereby

shortening the time of drying and materially reducing the time required for the carrotting treatment in its entirety.

Various changes in and departures from the embodiments of our carrotting composition may be made as the same have been hereinbefore exemplified, all within the scope and principles of our generic invention, and it is understood that the matter hereinbefore set forth is submitted as illustrative and not in a limiting sense.

We claim:

1. The process of preparing fur or the like for felting, which consists in subjecting the fur to the action of an aqueous carrotting solution of a substantially non-hydrolyzing oxidizing agent, a non-oxidizing acid capable of a substantial hydrolyzing action on the fur, and one or more non-oxidizing mercuric salts soluble in water of the group consisting of mercuric chloride, mercuric sulphate, mercuric ammonium chloride and double salts of the type  $K_2HgCl_4$ .

2. As a composition of matter for the carrotting of fur or the like, an aqueous carrotting solution containing a substantially non-hydrolyzing oxidizing agent, a non-oxidizing acid capable of a substantial hydrolyzing action on the fur, and one or more non-oxidizing mercuric salts soluble in water of the group consisting of mercuric chloride, mercuric sulphate, mercuric ammonium chloride and double salts of the type  $K_2HgCl_4$ .

3. As a composition of matter for the carrotting of fur or the like, an aqueous solution containing an oxidizing agent, a non-oxidizing acid capable of a substantial hydrolyzing action on the fur, and one or more non-oxidizing mercuric salts soluble in water of the group consisting of mercuric chloride, mercuric sulphate, mercuric ammonium chloride and double salts of the type  $K_2HgCl_4$ , said solution having the proportions represented by 100 parts by weight of water, from 8 to 25 parts by weight of said acid, and from 1 to 8 parts by weight of mercuric salt.

CONSTANTINE F. FABIAN.

ALEXANDER N. SACHANEN.

45

#### CERTIFICATE OF CORRECTION.

Patent No. 2,052,873.

September 1, 193

CONSTANTINE F. FABIAN, ET AL.

It is hereby certified that error appears in the printed specification of the above numbered patent requiring correction as follows: Page 4, second column, line 33, claim 3, strike out "an" and insert instead the words a substantially non-hydrolyzing; and that the said Letters Patent should be read with this correction therein that the same may conform to the record of the case in the Patent Office.

Signed and sealed this 13th day of October, A. D. 1936.

Henry Van Arsdale  
Acting Commissioner of Patents.

(Seal)

CERTIFICATE OF CORRECTION.

September 1, 193

Patent No. 2,052,873.

CONSTANTINE F. FABIAN, ET AL.

It is hereby certified that error appears in the printed specification of the above numbered patent requiring correction as follows: Page 4, second column, line 33, claim 3, strike out "an" and insert instead the words a substantially non-hydrolyzing; and that the said Letters Patent should be read with this correction therein that the same may conform to the record of the case in the Patent Office.

Signed and sealed this 13th day of October, A. D. 1936.

Henry Van Arsdale  
Acting Commissioner of Patents.

(Seal)